

2,825,643

## PROCESS FOR RECOVERY OF PLATINUM FROM PERCHLORATE CELL ELECTROLYTE

Joseph B. Heitman, Tacoma, Wash., assignor to Pennsalt Chemicals Corporation, a corporation of Pennsylvania

No Drawing. Application July 13, 1953  
Serial No. 367,731

9 Claims. (Cl. 75—108)

This invention relates to a new method of recovering platinum from solutions or suspensions in which platinum is present in only a very small concentration.

Platinum has heretofore been recovered from mixtures in which it is present in a minor amount by forming a soluble compound of platinum, for example, a chloroplatinate, and thereafter precipitating metallic platinum either by electrolytic means or by reduction with a metal such as zinc or magnesium. These methods are not efficient when the platinum is present in a quantity less than 0.01% by weight of the solution and are essentially ineffective when the platinum is present in still smaller amounts.

The electrolysis of sodium chlorate to sodium perchlorate is an example of a process where the present invention finds ready application. In this process, it is the present practice to use platinum anode surfaces in the electrolytic cells and, while platinum is almost completely inert to most acids, with the exception of aqua regia, there is a slow loss of platinum from anode surfaces during perchlorate electrolysis. This loss is both chemical and physical and amounts to from 5 to 15 grams of platinum per ton of sodium perchlorate produced, depending upon the conditions of electrolysis and the physical condition of the anodes. The platinum from the chemical dissolution is probably present in the liquor either as chloroplatinic acid ( $H_2PtCl_6$ ) or as sodium chloroplatinate. Platinum also may be lost as a result of physical erosion by gas bubbles and liquor and in this case the platinum is in the form of very fine colloidal particles. There are also larger pieces of platinum foil present, resulting from mechanical breakage of anodes which have been worn thin.

In accordance with the present invention, it has been found that chloroplatinates are either adsorbed on or will react with insoluble hydroxides of the flocculent or gelatinous type, such as the hydroxides of iron, nickel, cobalt and aluminum, and that this reaction or adsorption is substantially more complete when carried out in the presence of alkaline earth metal cations of group two of the periodic table. Examples of these are the cations of barium, strontium, and calcium.

Generally speaking, in the treatment of sodium perchlorate solutions, or other solutions containing platinum in very small amount, for the recovery of the platinum, a flocculent metal hydroxide precipitate, such as ferric hydroxide, may be formed in the sodium perchlorate solution. Ferric hydroxide is admirably suited for this purpose since there is some ferric hydroxide already present in perchlorate cell liquor due to corrosion of the cells, and ferric hydroxide is also easily separated from the perchlorate solution by filtration. If insufficient iron is present in the electrolyte for the precipitation of the platinum, additional iron may be added in the form of ferric chloride, which may be subsequently converted to ferric hydroxide by the addition of sodium hydroxide to the solution.

A cation as above defined must also be present in addi-

tion to the flocculent precipitate. The metallic cation may be added as a soluble salt; for example, when the cation is barium, barium chloride may be added. Perchlorate cell liquor normally contains sodium dichromate, and the addition of barium chloride precipitates barium chromate, thereby removing the chromate which was formerly present in the perchlorate solution as sodium dichromate. Since chromates are soluble to some extent in mineral acids, it is necessary that an alkaline condition be established before precipitation.

10 Ferric hydroxide is precipitated together with barium chromate upon adjustment of the pH of the solution to a value above 7. One of the results of the barium chloride addition, as previously noted, is the precipitation of chromate, but it has been found that only a very small amount of platinum is precipitated with the ferric hydroxide, or other flocculent precipitate, unless an excess of barium chloride, or other metallic cation, is present over that stoichiometrically required to precipitate the chromate. It is necessary to add the barium chloride, or other metallic cation, until the solution becomes water white, and this end point can be clearly seen in a strong light.

15 The co-precipitation may involve either a simple adsorption or a chemical reaction, but it is believed that in the case of the barium chloride-ferric hydroxide system, for example, a true chemical reaction takes place. This is indicated by the fact that ferric hydroxide will turn a brighter red color if a very small amount of a chloroplatinate salt is added to it in an aqueous solution. It is possible, therefore, that a compound of the general formula  $BaPtCl_6 \cdot Fe(OH)_3 \cdot yH_2O$  is formed. The reaction which forms this compound appears to be somewhat reversible, however, since chloroplatinates have been observed to go back into solution from a treated cell liquor. This reversal of the reaction may be prevented by immediate filtration of the sludge or by having a greater amount of barium chloride present.

20 After separating the sludge from the perchlorate liquor, the sludge is boiled, in the form of a thick slurry, with aqua regia until all of the metallic platinum is converted to chloroplatinates and all of the chromate is converted to trivalent chromium. A treatment sufficient to accomplish the latter will also be sufficient to accomplish the former. The residue from this treatment is then baked at an elevated temperature in order to convert all of the chloroplatinates to soluble salts which are believed to be chloroplatinates. The chloroplatinates may then be removed from the baked residue by boiling or leaching the residue with hot water containing a small quantity of hydrochloric acid.

25 The hot leach liquor is filtered to remove any suspended solid particles of residue and is then made alkaline to precipitate the hydroxides of iron and chromium. These precipitates are then filtered off, leaving a pale yellow solution of sodium, barium or other chloroplatinate. The color of this solution is dependent to a large extent on the pH thereof and becomes much paler at pH values below 7. The color of the solution is not an indication of the amount of platinum present.

30 Since the final liquor contains barium chloride and probably other dissolved salts, the platinum salts cannot be isolated by simple evaporation. Platinum, being a noble metal, is easily reduced by other metals, such as zinc, cadmium, magnesium, or aluminum in an acidified solution.

35 In a preferred mode of operation, platinum may be recovered from sodium perchlorate cell liquor by the following procedure: Sufficient ferric chloride is added to the perchlorate cell liquor to bring the ferric ion concentration to a value equivalent to about 0.5 gram per liter of ferric chloride, and the pH of the solution is adjusted

to about 8.0 with sodium hydroxide. An excess of barium chloride over that necessary to precipitate the chromate in the cell liquor is then added. The barium chloride, generally added as the dihydrate, requirement of the liquor is about 2 to 3 grams per liter. The point at which the platinum has precipitated may be determined by a filtration of a small sample and examination thereof for a water-white color. Chloroplatinates are very highly colored and small amounts thereof will lend a yellow tinge to aqueous solutions. This color may be detected by careful visual examination. Precipitation of chromate and ferric hydroxide will be accelerated if the temperature of the liquor is raised to about 80° C.

The precipitate is then filtered off and the sodium perchlorate liquor may then be treated, if necessary, with sodium carbonate to remove any excess barium. The precipitate, which will amount to about 3 gallons of wet sludge per ton of sodium perchlorate produced, is placed in an evaporating dish having two or three times as much depth as is occupied by the precipitate, since there is some frothing on boiling. The precipitate is moistened with aqua regia and boiled, with occasional stirring and acid addition, until all of the chromate is reduced to trivalent chromium, as evidenced by a dark spinach-green color. Chromates must be removed as they interfere with the final reduction of the platinum.

The residue is then transferred to an oven and baked at a temperature in the range of about 300 to 350° C. for about an hour after the interior of the residue becomes heated to about 300° C. at least. The baked residue is then ground to a powder and transferred to a tank containing about 10 times the volume of the residue, i. e., about 10 gallons, per ton of perchlorate produced, of hot water containing about 0.8% of hydrochloric acid, and the mixture is boiled for about 15 to 20 minutes. The mixture is then filtered, using a filter aid, and washed. The filtrate is retained.

The filtrate is made slightly alkaline, to a pH of about 8.0, with sodium hydroxide and the resulting ferric and chromic hydroxides are filtered off. The filtrate, which is a pale yellow in color, is retained and made slightly acid by the addition of hydrochloric acid, or other acid. A more reactive metal than platinum, such as magnesium, in the form of powder or sheet, is added to the acidic filtrate and the resulting reaction is permitted to proceed to completion, as evidenced by a water-white color in the liquor. Additional metal and acid may be added, if necessary, and best results are obtained if the mixture is agitated. The pH must be maintained at all times on the acid side but a large excess of acid should be avoided.

Upon completion of the reaction, the liquor is brought to boiling temperature to coagulate the platinum particles and to insure the dissolution of the more reactive reducing metal. The platinum, in the form of a pure, finely divided black powder, is then removed from the liquor by filtration.

It is understood that the foregoing description is illustrative only and variations therein may be made if desired. For example, the baking temperature for converting the chloroplatinates to chloroplatinites may be in the range of about 250 to 580° C. and the heating may be continued for about 0.5 to 8 hours. Similarly, leaching of the baked residue may be effected at a temperature of about 70 to 100° C. for about 15 to 60 minutes. Also, platinum may be recovered in metallic form from the soluble salts thereof by chemical or electrolytic reduction.

The invention will be further illustrated by reference to the following specific examples:

#### Example 1

One liter of a solution was prepared containing 750 grams of sodium perchlorate, 3 grams of sodium chloride, 0.5 gram of calcium chloride, 1 gram of sodium dichro-

mate, and 0.0104 gram of platinum, as an equivalent amount of potassium chloroplatinate.

0.5 gram of ferric chloride was dissolved in the solution and the solution was made alkaline with sodium hydroxide to precipitate ferric hydroxide. Sufficient barium chloride was added to precipitate the chromate and then an excess of barium chloride was added until all of the platinum was reacted with and/or adsorbed on the ferric hydroxide, as shown by an absence of color in the solution. The barium chloride dihydrate requirement was 3 grams. The solution was then filtered to remove the precipitate, which was then boiled with aqua regia until all of the chromate was reduced, and was then baked at a temperature of 300 to 350° C. for one hour to convert the platinum to a soluble form, believed to be chloroplatinite salts. The residue was then ground and boiled in water, containing 0.8% hydrochloric acid, to dissolve soluble salts and was then filtered. The filtrate was made alkaline to remove hydroxides of iron and chromium and was again filtered. The final filtrate contained soluble chloroplatinite salts, from which the platinum was recovered in metallic form by acidifying the filtrate and reducing the resulting acid compounds of platinum by the addition of magnesium sheet. The recovery of metallic platinum was 0.0092 gram, which is equivalent to an 89% recovery of the platinum in solution.

#### Example 2

25 liters of sodium perchlorate electrolyte, produced by the electrolysis of sodium chloride to sodium perchlorate, and having a composition similar to that of the solution of Example 1 except for the quantity of platinum, which in this case was 0.5235 gram of platinum, primarily in solution, were treated in accordance with the procedure of Example 1, with the exception that no ferric salts were added, since sufficient iron was already present as a result of corrosion of the electrolytic cell. 0.4810 gram of metallic platinum was recovered, which is a recovery of 91.9%.

Prior to the present invention, the recovery of platinum lost from anodes in the electrolytic manufacture of sodium perchlorate was limited to platinum in metallic form, which was present in pieces large enough to be filtered from the electrolyte or cell mud. The present invention provides a method for the recovery of finely divided platinum or platinum salts from perchlorate cell liquor and other dilute solutions. Also, in the present process only a slight quantity of additional materials is added to the cell liquor, hence there is no contamination thereof and consequently no extra purification steps are required.

It will be obvious to those skilled in the art that many modifications may be made within the scope of the present invention without departing from the spirit thereof, and the invention includes all such modifications.

55 I claim:

1. The method of recovering platinum from perchlorate cell electrolyte which comprises forming a flocculent metal hydroxide precipitate in the said electrolyte in the presence of an alkaline earth metal cation added in excess of the stoichiometric amount required to precipitate the anions present in the said electrolyte, which are reactive with alkaline earth metal cations, separating the resulting precipitate, and recovering metallic platinum therefrom.

60 2. The process of claim 1 in which the metal hydroxide is selected from the group consisting of ferric, nickel, cobalt and aluminum hydroxides.

3. The method of claim 1 in which the metal hydroxide is ferric hydroxide.

70 4. The method of claim 1 in which the alkaline earth metal cation is barium.

5. The method of recovering platinum from perchlorate cell electrolyte containing minute amounts of platinum as well as small amounts of chromate ion which 75 comprises adding alkali to adjust the pH of the said

electrolyte to in excess of 7, adding alkali earth metal cations in excess of the amount necessary to precipitate all of the chromate present in the said electrolyte, forming flocculent metal hydroxide precipitate in the presence of an excess of the said alkali earth metal cation, separating the resulting precipitate from the liquor and recovering metallic platinum therefrom.

6. The method of claim 5 in which the alkali earth metal cation is barium.

7. The method of claim 5 in which ferric chloride is added to the perchlorate cell electrolyte until its concentration is about 0.5 gram per liter, the said addition being made prior to the addition of the alkali earth metal cation.

8. The method of claim 5 in which the addition of the alkali metal cation is continued until a filtered portion of the treated electrolyte is water-white in color.

9. The method of recovering platinum from perchlorate cell electrolyte containing minute amounts of platinum as well as small amounts of chromate ion which comprises adding alkali to adjust the pH of the said electrolyte to an excess of 7, adding an alkali earth metal cation in excess of the amount necessary to precipitate

all of the chromate present in the said electrolyte, and forming flocculent metal hydroxide precipitate in the presence of an excess of the said alkali earth metal cation.

5

References Cited in the file of this patent

UNITED STATES PATENTS

|           |          |                |
|-----------|----------|----------------|
| 1,797,879 | Rudolfs  | Mar. 24, 1931  |
| 1,876,943 | Hull     | Sept. 13, 1932 |
| 2,086,384 | Lady     | July 6, 1937   |
| 2,131,045 | Hickman  | Sept. 27, 1938 |
| 2,344,429 | Gelder   | Mar. 14, 1944  |
| 2,542,743 | Weymouth | Feb. 20, 1951  |

OTHER REFERENCES

Kolthoff et al.: "Textbook of Quantitative Inorganic Chemistry," The MacMillan Co., New York, rev. ed. (1946).

20 Sandell: "Colorimetric Determination of Traces of Metals," Interscience Publishers, Inc., New York, 2nd ed. (1950), pages 20-27 and page 494. (Copies of above pub. in Sci. Lib.)